

# UNITED STATES PATENT OFFICE

EDMOND ALEXANDRE PRETCEILLE, OF NANTES, FRANCE, ASSIGNOR TO THE CORPORATION OF METALLURGISCHE GESELLSCHAFT A. G., OF FRANKFORT-ON-THE-MAIN, GERMANY.

## PROCESS OF AGGLOMERATING FINE ORES OR METALLIFEROUS PRODUCTS.

1,096,054.

Specification of Letters Patent.

Patented May 12, 1914.

No Drawing.

Application filed October 4, 1910. Serial No. 585,226.

*To all whom it may concern:*

Be it known that I, EDMOND ALEXANDRE PRETCEILLE, of Ile Ste. Anne, in the city of Nantes, France, a citizen of the Republic 5 of France, have invented certain new and useful Improvements in Processes of Agglomeration of Fine Ores or Metalliferous Products, of which the following is a specification.

- 10 In the U. S. Patent No. 844,355 of Ferdinand Heberlein, there is disclosed a method of sintering fine ores or metalliferous products according to which the ore, mixed with fuel, is exposed to the action of 15 a current of air, with the result, that the ore is reduced to sinter in consequence of the heat produced by the combustion of the fuel. When this method is employed, the major portion of the fine ore is in most 20 cases sintered in the form of a homogeneous block, and only a relatively small percentage of the ore—5 to 10 per cent.—remains unsintered. It is often possible to increase the proportion of sintered material and to 25 diminish the time occupied in treating a charge by adding water to the mixture of ore and coal. In the working of certain ores, especially certain kinds of pyrites residues, and dust-like products of the blast-furnace, the method above referred to, even 30 when water is added, fails to accomplish results which can be regarded as entirely satisfactory, too high a percentage of the material remaining unsintered. It would 35 appear, that the water quickly evaporates, leaves the ore loose and porous, and permits the air blast to sweep through the porous mass with great force, thus preventing the agglomeration of the particles.
- 40 My present invention is designed to obviate this defect. According to my improved method of working, the mixture of ore and fuel is moistened with a solution of a suitable salt hereinafter more particularly 45 referred to. When a salt solution is employed, it is probable that the water contained in the mass is retained by the salt until the combustion reaches the particular part affected. It may however, be that the 50 salt exercises upon the loose particles a cementing effect, so that only a restricted passage is allowed for the passage of the air blast.

The employment of sulfate of iron has been found particularly advantageous for 55 the purpose above referred to. Solutions of this salt are obtained in large quantities as refuse, as for example, in the freeing of pyrites cinders from copper. The employment of sulfate of iron has the further advantage that the agglomerate not only suffers no deterioration qualitatively, but is improved by reason of the salt being decomposed in the refining process, the sulfurous acid escaping while ferric oxid remains.

Instead of employing salt solutions, they can of course be formed in the material itself, by adding a suitable acid. If, in the case of an iron ore, sulfuric acid be added, 70 sulfate of iron is produced in the mass, or sulfate of manganese, in the case of a manganese ore. In like manner, alkali and earthy alkali sulfate and chlorids may be employed. These salts are decomposable at 75 sintering temperatures.

The degree of concentration of the salt solution to be employed, as also the quantity to be added, is readily determinable by experiment in respect to each particular ore. 80 As a rule, it is expedient to employ highly concentrated solutions, and to use such a quantity of the solution as to insure complete saturation of the mass. In the case of sulfate of iron solutions, 10° to 15° 85 Baumé have been found to yield good results.

Having now particularly described and ascertained the nature of my said invention and in what manner the same is to be performed, I claim:

1. In the process of sintering, the steps consisting in preparing a moistened mixture of finely divided metal-bearing material, fuel and a salt decomposable at sintering temperatures, igniting the mixture, and passing an air blast through it, substantially as described. 95
2. In the process of sintering, the steps consisting in preparing a moistened mixture of finely divided metal-bearing material, fuel, and a sulfate salt decomposable at sintering temperatures, igniting the mixture, and passing an air blast through it, substantially as described. 100
3. In the process of sintering, the steps 105

- consisting in preparing a moistened mixture of finely divided metal-bearing material, fuel and a sulfate of a metal decomposable at sintering temperatures, igniting 5 the mixture, and passing an air blast through it, substantially as described.
4. In the process of sintering, the steps consisting in preparing a moistened mixture of finely divided metal-bearing material, 10 fuel and sulfate of iron, igniting the mixture, and passing an air blast through it, substantially as described.
5. In the process of sintering finely divided metal-bearing material, the step consisting of passing an air blast through an ignited mass of such material, having adjacent to the blast exit surface a moistened mixture of the finely divided metal-bearing material, fuel, and a salt decomposable at sintering temperatures; substantially as described.
6. In the process of sintering a mixture of finely divided metal-bearing material and fuel by conducting a blast of air through the mixture after ignition, the method of preventing disturbance of the particles of the mixture by the air blast, which consists in binding the said particles with a sulfate salt

solution decomposable at sintering temperatures, substantially as described.

7. In the process of sintering a mixture of finely divided metal-bearing material and fuel by conducting a blast of air through the mixture after ignition, the method of preventing disturbance of the particles of the 30 particles of the mixture by the air blast, which consists in binding the said particles with a solution of a sulfate of a metal decomposable at sintering temperatures, substantially as described.

8. In the process of sintering a mixture of finely divided metal-bearing material and fuel by conducting a blast of air through the mixture after ignition, the method of preventing disturbance of the particles of the 35 mixture by the air blast, which consists in binding the said particles with a sulfate of iron solution, substantially as described.

In testimony whereof I have signed my name to this specification in the presence of 40 two subscribing witnesses.

EDMOND ALEXANDEE PRETCEILLE.

Witnesses:

RAOUL THOMJEAN,  
SAMUEL ALLEYNE.